

3,015,623

## LITHIUM BASE GREASE CONTAINING LEAD OLEATE, SULFURIZED LARD OIL AND MOLYBDENUM DISULFIDE

Lewis D. Loring, Dolton, and Henry J. Voss, Homewood, Ill., assignors to Sinclair Refining Company, New York, N.Y., a corporation of Maine

No Drawing. Filed June 24, 1960, Ser. No. 38,456

3 Claims. (Cl. 252—18)

The present invention relates to a grease composition of unusually high extreme pressure properties.

The increases in gear and bearing loading within recent years and the more vigorous service conditions in other instances of metal to metal contact have made extreme pressure lubricants and lubrication a limiting factor in performance. Much difficulty has been experienced in formulating greases capable of operating under severe conditions to protect effectively metal surfaces which come in contact with the lubricant. It is well known that the high pressure occurring in certain types of gears and bearings may cause a film of lubricant to rupture with subsequent damage to the machinery. It has been shown that lubricants can be improved with regard to their protective effect on rubbing surfaces by the addition of certain substances so that excessive wear, scuffing and seizure which normally follow a break in the film of lubricant can be prevented. Ingredients of this character are called extreme pressure (E.P.) ingredients. Numerous materials are known to impart extreme pressure properties to lubricants, as for instance, compounds containing sulfur, chlorine, phosphorous or lead. However, the simple presence of these elements does not guarantee extreme pressure properties and various compounds that do have these properties can vary considerably in their effectiveness.

We have now found that greases having incorporated therein small effective amounts of lead oleate, sulfurized lard oil, and molybdenum disulfide exhibit surprisingly high extreme pressure characteristics. The lead soap of the present invention is lead oleate. The amount of sulfur in the sulfurized lard oil will usually range from about 5 to 15%, preferably about 9 to 12% by weight.

The amount of the additives of this invention added to the grease is that sufficient to impart extreme pressure properties to the grease. Thus, the amount of the additives will vary depending on the particular characteristics of the grease utilized. In general about 2 to 4 weight percent of lead oleate will be employed. The amount of sulfurized lard oil utilized is usually about 3 to 6 weight percent, preferably about 4 to 5 weight percent. The molybdenum disulfide component of the present invention is generally employed in effective amounts of about 0.5 to 3 weight percent, preferably about 1 to 2 weight percent.

The grease employed with the novel additive combination of this invention can be a mineral lubricating oil base stock thickened to grease consistency with a lithium soap, for instance, a lithium soap of the ordinary saturated and unsaturated soap-forming fatty acids of about 12 to 20 carbon atoms including the hydrogenated fatty acids. Highly preferred soaps are the soap-forming hydroxy fatty acids, e.g. 12-hydroxy stearic acid, and their simple esters and glycerides, such as hydrogenated castor oil. The amount of soap employed is that sufficient to thicken the base oil to grease consistency. This amount is generally about 10 to 50 weight percent. The base oils thickened to grease consistency are of lubricating viscosity and can be petroleum lubricating oils derived from paraffinic, naphthenic, asphaltic or mixed based crudes. The oils may also be synthetic such as synthetic ester oils, e.g. di-2-ethylhexyl sebacate. The composi-

tion of the present invention can also contain other additives such as antioxidants, corrosion inhibitors, and anti-wear agents.

Lithium 12-hydroxy stearate-thickened greases prepared by in-situ soap formation and dehydration at a maximum temperature of about 300 to 350° F., e.g. 330° F., and containing the novel additive combination of the present invention were subjected to the Shell 4-ball wear test, the 4-ball extreme pressure test and the Timken test. These tests have been fully described in literature under the subject of anti-wear and extreme pressure testing. Thus, we will not go into detail concerning the procedure of each. The possible exception to the above is the Timken test. Details of this test can be found in U.S. Patent No. 2,715,612. The results of these tests are found in Table I.

Table I

|    | Grease Composition             | 1      | 2      | 3      | 4      |
|----|--------------------------------|--------|--------|--------|--------|
| 20 | Base Grease Ingredients:       |        |        |        |        |
|    | Hydrogenated Castor Oil        | 14.10  | 13.14  | 13.07  | 12.50  |
|    | Lithium Hydroxide              | 2.17   | 2.02   | 2.01   | 1.86   |
|    | 500 SUS at 100° F. Neutral Oil | 83.73  | 78.04  | 77.62  | 77.34  |
| 25 | Additives:                     |        |        |        |        |
|    | Lead Oleate                    |        | 2.30   | 2.30   | 2.30   |
|    | Sulfurized Lard Oil (12% S)    |        | 4.00   | 4.00   | 4.00   |
|    | MoS <sub>2</sub>               | .50    | 1.00   | 2.00   |        |
|    |                                | 100.00 | 100.00 | 100.00 | 100.00 |
| 30 | Unworked Pene                  | 277    | 286    | 298    | 278    |
|    | Worked Pene                    | 270    | 293    | 298    | 289    |
|    | Dropping Point, ° F.           | 384    | 365    | 364    | 367    |
|    | 4-Ball Wear Test, 640 r.p.m.   |        |        |        |        |
|    | 80° C.—15 kg.—2 Hr.            | 0.31   | 0.39   | 0.43   | 0.49   |
|    | Avg. Wear, mm.                 |        |        |        |        |
|    | 4-Ball EP Test—                |        |        |        |        |
|    | MHL                            | 20.0   | 45.0   | 55.8   | 67.4   |
|    | Weld, kg.                      | 141    | 224    | 251    | 251    |
| 35 | Timken Test—                   |        |        |        |        |
|    | Pass, lbs.                     | 3      | 45     | 60     | 70     |
|    | Fall, lbs.                     | 6      | 50     | 65     | 75     |

As demonstrated by the Timken pass load, the extreme pressure properties of the grease containing the three component additive combination of the present invention are superior greases.

Five samples of greases containing a total of 8.3% of additives (the total amount of additives used with 2% MoS<sub>2</sub> shown in Table I) were also tested. The results are shown in Table II.

Table II

|    | Grease Composition          | 1      | 2      | 3      | 4      |
|----|-----------------------------|--------|--------|--------|--------|
| 50 | Base Grease Ingredients:    |        |        |        |        |
|    | Hydrogenated Castor Oil     | 12.92  | 12.92  | 12.50  | 12.50  |
|    | Lithium Hydroxide           | 1.99   | 1.99   | 1.86   | 1.86   |
|    | 500 SUS at 100° F. Neutral  | 76.79  | 76.79  | 77.34  | 77.34  |
| 55 | Additives:                  |        |        |        |        |
|    | Sulfurized Lard Oil (12% S) | 5.27   |        | 4.00   |        |
|    | Lead Oleate                 | 3.03   |        |        | 2.30   |
|    | Sulfurized Sperm Oil        |        |        |        | 4.00   |
|    | Lead Naphthenate            |        |        | 2.30   |        |
|    | MoS <sub>2</sub>            |        | 8.30   | 2.00   | 2.00   |
|    |                             | 100.00 | 100.00 | 100.00 | 100.00 |
| 60 | Unworked Pene               | 286    | 280    | 286    | 290    |
|    | Worked Pene                 | 317    | 261    | 292    | 293    |
|    | Timken Test—                |        |        |        |        |
|    | Pass, lbs.                  | 30     | 15     | 30     | 24     |
|    | Fall, lbs.                  | 35     | 20     | 35     | 27     |

The data shows that none of the grease compositions of Table II has the high Timken pass load obtained by the three component additive combination of the present invention in a comparable total amount. Thus the data of Tables I and II clearly demonstrate that we have discovered a novel combination of additives that endows a grease with unexpectedly high extreme pressure properties. Also, the compositions containing lead naphthenate or sulfurized sperm oil demonstrated poor results when subjected to the Timken test.

We claim:

1. A grease composition of improved extreme pressure characteristics consisting essentially of a petroleum base lubricating oil thickened to grease consistency with lithium 12-hydroxy stearate soap, about 2 to 4 weight percent lead oleate, about 3 to 6 weight percent sulfurized lard oil and about 0.5 to 3 weight percent molybdenum disulfide.

2. The grease composition of claim 1 wherein the amount of molybdenum disulfide is about 1 to 2 weight percent.

3. The grease composition of claim 2 wherein the

amount of sulfurized lard oil is about 4 to 5 weight percent.

References Cited in the file of this patent

UNITED STATES PATENTS

|           |               |                |
|-----------|---------------|----------------|
| 2,156,803 | Cooper et al. | May 2, 1939    |
| 2,449,510 | Robertson     | Sept. 14, 1948 |
| 2,609,343 | White et al.  | Sept. 2, 1952  |
| 2,858,273 | Worth         | Oct. 28, 1958  |
| 2,898,297 | Schott        | Aug. 4, 1959   |

UNITED STATES PATENT OFFICE  
CERTIFICATE OF CORRECTION

Patent No. 3,015,623

January 2, 1962

Lewis D. Loring et al.

It is hereby certified that error appears in the above numbered patent requiring correction and that the said Letters Patent should read as corrected below.

Column 4, line 8, for "2,609,343" read -- 2,609,342 --.

Signed and sealed this 24th day of July 1962.

(SEAL)

Attest:

ERNEST W. SWIDER  
Attesting Officer

DAVID L. LADD  
Commissioner of Patents